

[54] TALC-MOLYBDENITE SEPARATION

|         |        |                     |         |
|---------|--------|---------------------|---------|
| 19,374  | 9/1915 | United Kingdom..... | 209/167 |
| 19,731  | 4/1929 | Australia.....      | 209/167 |
| 522,712 | 3/1956 | Canada.....         | 209/167 |

[75] Inventors: **Richard O. Huch; Pedro Valles,**  
both of Tucson, Ariz.[73] Assignee: **Pima Mining Company, Los**  
Angeles, Calif.[22] Filed: **Sept. 27, 1973**[21] Appl. No.: **401,151****Related U.S. Application Data**[63] Continuation-in-part of Ser. No. 216,723, Jan. 10,  
1972, abandoned.[52] U.S. Cl. .... **209/167**[51] Int. Cl.<sup>2</sup> .... **B03D 1/06**[58] Field of Search..... **209/166, 167**[56] **References Cited****UNITED STATES PATENTS**

|           |         |               |           |
|-----------|---------|---------------|-----------|
| 1,102,738 | 7/1914  | Greenway..... | 209/167   |
| 1,397,703 | 11/1921 | Robbins.....  | 209/167   |
| 2,255,776 | 9/1941  | Janney.....   | 209/166 X |
| 2,492,936 | 12/1949 | Nokes.....    | 209/167   |
| 2,620,068 | 12/1952 | Allen.....    | 209/167   |
| 3,313,412 | 4/1967  | Bloom.....    | 209/167   |

**FOREIGN PATENTS OR APPLICATIONS**

6,887 4/1932 Australia..... 209/166

19,374 9/1915 United Kingdom..... 209/167

19,731 4/1929 Australia..... 209/167

522,712 3/1956 Canada..... 209/167

**OTHER PUBLICATIONS**

50th Anniv. Vol., Froth Flotation, 1962, 393-398.

Chem. Abstracts, Vol. 69, 1968, 98563 h.

Chem. Abstracts, Vol. 69, 1968, 10208, 108806 f.

Chem. Abstracts, Vol. 71, 1969, 23841 e.

*Primary Examiner*—Robert Halper*Attorney, Agent, or Firm*—Elwood S. Kendrick

[57]

**ABSTRACT**

A method of enriching the molybdenite fraction of ores and concentrates having hydrophobic silicates containing magnesium such as talc. An aqueous slurry of the ore or concentrate is treated with a water soluble metallic salt of a weak base and strong acid and a water soluble salt of a weak acid and subjected to agitation. The treated pulp is then subjected to a conventional froth flotation wherein a molybdenite fraction is floated off as molybdenite enriched concentrate and a talc fraction is depressed into the tailings.

**22 Claims, No Drawings**

**TALC-MOLYBDENITE SEPARATION**

This application is a continuation-in-part of our co-pending patent Application Ser. No. 216,723, now abandoned, filed Jan. 10, 1972.

**BACKGROUND OF THE INVENTION**

This invention is directed to a process for separating hydrophobic silicates containing magnesium known as talc for molybdenite bearing ores and concentrates. In particular this invention is directed to a flotation process for molybdenite ores and concentrates where a hydrophobic talc fraction is depressed and the molybdenite fraction is selectively floated away therefrom.

Lack of a commercial process emphasizes the difficulty of selectively floating molybdenite from molybdenite bearing concentrates having hydrophobic silicates containing magnesium such as talc. Organic colloids or organic dyes have been used for the upgrading of molybdenite concentrates and ores, but in such applications both the molybdenite and the contaminants could be depressed. The presence of talc is undesirable because it complicates the further treatment of molybdenite.

The effective commercial methods for upgrading molybdenite from molybdenite bearing concentrates having hydrophobic silicates containing magnesium are those related to the Utah Process whereby bulk molybdenite bearing concentrates are either roasted or spray dried to render the molybdenum less floatable than acid insoluble contaminants including hydrophobic silicates containing magnesium. These contaminants are then floated leaving a molybdenite enriched tailing.

These processes require expensive and elaborate systems of multiple hearth roasters or spray dryers with adequate dust collecting systems. Temperature, retention time, and degree of oxidation of the minerals are very critical. The expenditure of energy for heat and transportation of the ore concentrate is costly. The roasting process has been used at the Pima Mining Company, on final molybdenite concentrates. Other properties use more bulky concentrates from the initial stages of their molybdenite recovering plants.

**SUMMARY OF THE INVENTION**

The present process consists of treating pulps of molybdenite bearing concentrates having a substantial amount of hydrophobic silicates containing magnesium by agitation in the presence of a water soluble metallic salt of a weak base and a strong acid and a water soluble salt of a weak acid. The treated pulp is then subjected to a conventional froth flotation wherein a molybdenite fraction is floated off as a molybdenite enriched concentrate and hydrophobic silicate containing magnesium, such as talc, is depressed into the tailings.

The subject process is useful in that there is sufficient depression of hydrophobic silicates containing magnesium, so that either a marketable grade of molybdenite concentrate is produced directly or the molybdenite concentrate is enriched so that subsequent processing is facilitated.

**DESCRIPTION OF THE INVENTION**

The present process is practiced by preparing aqueous slurry or pulp of ground molybdenite concentrate or a molybdenite bearing ore. Generally the concentrated ore is ground to minus 10 mesh, preferably minus 48 mesh. The pulp density varies between about

1% and about 45% solids; however, our tests of the process indicate that a more satisfactory separation is obtained at 5% to 15% solids.

The pulp is then treated with a water-soluble metallic salt of a weak base and a strong acid and a water-soluble salt of a weak acid. Between about 1 and about 30 pounds of the metallic salt of the weak base and strong acid are used per each ton of solids. Between about 1 and about 45 pounds of the salt of the weak acid are used per ton of solids. Optimum salt concentrations are dependent upon pulp conditions and salt combinations.

Best results are usually obtained if the pulp is treated first with the metallic salt of a weak base and a strong acid and then followed by the addition of the salt of a weak acid prior to flotation. However, satisfactory results can be obtained when the salt of a weak acid is added first, followed by the addition of the metallic salt of a weak base and a strong acid; both salts are added simultaneously; or both salts are premixed and then added to the pulp.

The preferred metallic salts of a weak base and strong acids are the water-soluble sulfate, nitrate, fluoride and chloride salts of aluminum, manganese, calcium, magnesium, zinc, copper, cobalt, nickel, chromium, iron and cadmium.

Typical salts of weak acids that can be employed in the present process include the water-soluble alkali metal (especially sodium and potassium), ammonium, and alkaline earth metal (especially calcium and magnesium) salts of silicic acids; carbonic acid; acids of phosphorus, including phosphoric acid, hypophosphorous acid, phosphorous acid, hypophosphoric acid and the like; the acids of boron, including ortho-boric acid, meta boric acid, tetraboric acid and the like; and hydroferrocyanic acid but only when the aforesaid metallic salt is a water-soluble salt of zinc. It will be appreciated by reference to chemical handbooks that not all of the possible combinations of the above are water-soluble.

The pulp and salts are agitated for a period of from about 1 minute to about 60 minutes, preferably about 30 minutes. Then the pulp is subject to a conventional froth flotation for about 1 to about 30 minutes. The molybdenite fraction is floated off as an enriched molybdenite concentrate. The molybdenite recovery is very high, from about 80 to about 96% and the concentrate can be enriched by a factor of about 2 to about 5 times. The hydrophobic silicates fraction and other acid insoluble contaminants are depressed into the tailings (from about 50 to about 85% of the acid insoluble contaminants, principally talc and other hydrophobic silicates, are depressed into the tailings).

The following examples are intended to further illustrate the present invention and not intended as limitations thereof. Naturally the process conditions such as process times, temperature, pH and reagent concentration can be varied through routine experimentation to optimize the end results for a particular ore, mesh size, pulp density, and particular reagents employed.

**EXAMPLE 1 (NO TREATING AGENT)**

A composite sample of low grade molybdenite concentrate produced at the Pima Mine containing approximately 18% molybdenite, 4% chalcopyrite, 5% pyrite and 69% acid insoluble minerals was made into a dilute pulp of five percent solids in water at ambient temperature in a laboratory flotation cell. A major portion of the said acid insoluble minerals was a hydropho-

bic silicate containing magnesium, i.e., talc. The pulp was immediately subjected to froth flotation and the froth removed for five minutes, during which a concentrate was separated. This example is given to exemplify the response of the composite sample without treatment by our new process. The results of the example are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 10.98   | 68.8   | 100.0                | 100.0  |
| Concentrate | 93.75          | 11.35   | 68.9   | 96.9                 | 3.9    |
| Tailing     | 6.25           | 5.47    | 66.7   | 3.1                  | 6.1    |

### EXAMPLE 2

Another sample of the same composite described in example 1 was subjected to the pulping procedure described in example 1. The pulp was then agitated with a quantity of zinc sulfate corresponding to four pounds per ton of solids for thirty minutes. A quantity of sodium silicate corresponding to 7.5 pounds per ton of solids was then added. The pulp was then subjected to flotation as described in example 1. The results are presented in the following table, showing the beneficial results obtainable by use of our method.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 10.98   | 67.7   | 100.0                | 100.0  |
| Concentrate | 44.69          | 22.53   | 49.7   | 89.0                 | 32.8   |
| Tailing     | 55.31          | 2.24    | 82.2   | 11.0                 | 67.2   |

### EXAMPLE 3

Still another sample of the same composite described in example 1 was subjected to the pulping procedure described in example 1. A quantity of sodium silicate corresponding to 7.5 pounds per ton of solids was added to the pulp. A quantity of zinc sulfate corresponding to 16 pounds per ton of solids was then added to the pulp. The pulp was agitated for thirty minutes and then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 10.99   | 67.5   | 100.0                | 100.0  |
| Concentrate | 54.08          | 19.03   | 55.1   | 93.6                 | 44.1   |
| Tailing     | 45.92          | 1.53    | 82.2   | 6.4                  | 55.9   |

### EXAMPLE 4

A sample of the composite described in example 1 was subjected to the pulping procedure described in example 1. A quantity of 10% sodium silicate solution was placed in a beaker. To this was added a quantity of 10% zinc sulfate solution. The contents in the beaker were then washed into the pulp. The quantity of sodium silicate corresponded to 7.5 pounds per ton of solids; the quantity of zinc sulfate corresponded to 16 pounds per ton of solids. The pulp was agitated for thirty min-

utes and then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.0          | 11.10   | 68.2   | 100.0                | 100.0  |
| Concentrate | 56.61          | 18.12   | 58.0   | 92.4                 | 48.1   |
| Tailing     | 43.39          | 1.95    | 81.6   | 7.6                  | 51.9   |

### EXAMPLE 5

A sample of the composite described in example 1 was subjected to the pulping procedure described in example 1. The pulp was then agitated with a quantity of zinc sulfate corresponding to 16 pounds per ton of solids for thirty minutes. An addition of disodium hydrogen phosphate corresponding to 7.5 pounds per ton of solids was then added. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.0          | 10.97   | 68.1   | 100.0                | 100.0  |
| Concentrate | 35.56          | 28.58   | 40.1   | 92.6                 | 20.9   |
| Tailing     | 64.44          | 1.26    | 83.6   | 7.4                  | 79.1   |

### EXAMPLE 6

A sample of the composite described in example 1 was subjected to the pulping procedure described in example 1. The pulp was then agitated with a quantity of zinc sulfate corresponding to 16 pounds per ton of solids for thirty minutes. An addition of sodium acid carbonate corresponding to 7.5 pounds per ton of solids was then added. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 11.66   | 67.6   | 100.0                | 100.0  |
| Concentrate | 33.94          | 32.56   | 35.2   | 94.8                 | 17.7   |
| Tailing     | 66.06          | 0.92    | 84.2   | 5.2                  | 82.3   |

### EXAMPLE 7

A sample of the composite described in example 1 was subjected to the pulping procedure described in example 1. A quantity of 10% sodium silicate solution was placed in a beaker. To this was added a quantity of 10% aluminum sulfate solution. The contents in the beaker were then washed into the pulp. The quantity of sodium silicate corresponded to 7.5 pounds per ton of solids; the quantity of aluminum sulfate corresponded to six pounds per ton of solids. The pulp was then agitated for thirty minutes and then subjected to flotation as described in example 1. The results are presented in the following table:

-continued

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 10.52   | 68.3   | 100.0                | 100.0  |
| Concentrate | 52.50          | 17.59   | 58.0   | 87.8                 | 44.6   |
| Tailing     | 47.50          | 2.71    | 79.7   | 12.2                 | 55.4   |

## EXAMPLE 8

A sample of the composite described in example 1 was subjected to the pulping procedure described in example 1. The pulp was then agitated with a quantity of aluminum sulfate corresponding to two pounds per ton of solids for five minutes. A quantity of disodium hydrogen phosphate corresponding to 7.5 pounds per ton of solids was then added. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 10.91   | 68.8   | 100.0                | 100.0  |
| Concentrate | 42.45          | 21.29   | 51.6   | 82.8                 | 31.8   |
| Tailing     | 57.55          | 3.26    | 81.5   | 17.2                 | 68.2   |

## EXAMPLE 9

A sample of the composite described in example 1 was subjected to the pulping procedure described in example 1. The pulp was then agitated with a quantity of aluminum sulfate corresponding to one pound per ton of solids for two minutes. A quantity of sodium acid carbonate corresponding to 7.5 pounds per ton of solids was then added. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 10.99   | 68.6   | 100.0                | 100.0  |
| Concentrate | 52.51          | 18.82   | 55.6   | 89.9                 | 42.6   |
| Tailing     | 47.49          | 2.34    | 82.9   | 10.1                 | 57.3   |

## EXAMPLE 10

A sample of the composite described in example 1 was subjected to the pulping procedure described in example 1. The pulp was then agitated with a quantity of chromic sulfate corresponding to four pounds per ton of solids for five minutes. A quantity of sodium silicate corresponding to 7.5 pounds per ton of solids was then added to the pulp. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 11.17   | 69.1   | 100.0                | 100.0  |
| Concentrate | 34.09          | 29.66   | 41.7   | 90.4                 | 20.6   |

| Product | Weight Percent | Percent |        | Distribution Percent |        |
|---------|----------------|---------|--------|----------------------|--------|
|         |                | Mo      | Insol. | Mo                   | Insol. |
| Tailing | 65.91          | 1.62    | 83.3   | 9.6                  | 79.4   |

## EXAMPLE 11

A sample of the composite described in example 1 was subjected to the pulping procedure described in example 1. The pulp was then agitated with a quantity of chromic sulfate corresponding to four pounds per ton of solids for five minutes. A quantity of disodium hydrogen phosphate corresponding to 7.5 pounds per ton of solids was then added to the pulp. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 11.34   | 69.4   | 100.0                | 100.0  |
| Concentrate | 56.21          | 18.36   | 30.4   | 91.0                 | 48.9   |
| Tailing     | 43.79          | 2.32    | 81.0   | 9.0                  | 51.1   |

## EXAMPLE 12

A sample of the composite described in example 1 was subjected to the pulping procedure described in example 1. The pulp was then agitated with a quantity of chromic sulfate corresponding to four pounds per ton of solids for five minutes. A quantity of sodium acid carbonate corresponding to 7.5 pounds per ton of solids was then added to the pulp. The pulp was then subjected to flotation as described in example 1. The results are presented in the following table.

| Product     | Weight Percent | Percent |        | Distribution Percent |        |
|-------------|----------------|---------|--------|----------------------|--------|
|             |                | Mo      | Insol. | Mo                   | Insol. |
| Head        | 100.00         | 11.39   | 69.2   | 100.0                | 100.0  |
| Concentrate | 51.38          | 20.28   | 56.4   | 91.5                 | 41.9   |
| Tailing     | 48.62          | 1.99    | 82.8   | 8.5                  | 58.1   |

## EXAMPLE 13

The procedure of example 2 is repeated employing a pulp density of about 5% solids,  $MnCl_2$  (16 pounds per ton of solids) in place of  $ZnSO_4$  and sodium silicate (7.5 pounds per ton of solids) with good results.

## EXAMPLE 14

The procedure of example 9 is repeated with a pulp density of about 1% solids and the water-soluble calcium salts of boron (3 pounds per ton of solids) with similar results.

## EXAMPLE 15

Another sample of a low grade molybdenite concentrate that contained a substantial portion of a hydrophobic talc was made into a dilute pulp of approximately 5% solids in water at ambient temperature in a laboratory flotation cell. This pulp had a pH of 8.3. The sample so prepared was then agitated with a quantity of

zinc sulfate corresponding to six pounds per ton of solids for about 30 minutes. The pH of this admixture was measured and found to be 6.8. Thereafter one pound per ton of solids of NaOH was mixed with the pulp so treated resulting in a pH of 7.1. Thereafter eight pounds per ton of potassium ferrocyanide was mixed with the aforementioned pulp containing zinc sulfate and NaOH. The resulting admixture had a pH of 8.2. The said admixture was immediately subjected to froth flotation and the froth removed for five minutes during which a concentrate was separated with results as follows.

| Percent Weight in Concentrate | Head | Percent Mo In Tail | Concentrate | Percent Mo Recovered in Concentrate |
|-------------------------------|------|--------------------|-------------|-------------------------------------|
| 19.9                          | 4.13 | 0.23               | 19.88       | 95.5                                |

The benefits from the above processing will be appreciated by comparing said results with the following wherein the said pulp made up to 5% solids was floated without the addition of our new treating reagents, i.e., such as zinc sulfate and potassium ferrocyanide.

| Percent Weight in Concentrate | Head | Percent Mo in Tail | Concentrate | Percent Mo Recovered in Concentrate |
|-------------------------------|------|--------------------|-------------|-------------------------------------|
| 98.1                          | 4.66 | 1.34               | 4.73        | 99.4                                |

As a result of repeating the above experiment substituting various metals for zinc, it was observed that no effective separation of talc from a molybdenite bearing concentrate was obtained.

#### EXAMPLE 16

##### Method of Determining Acid Insoluble Percentage in Molybdenite Containing Ore or Concentrate.

###### Procedure:

1. Weight 0.5 gram of molybdenum concentrate sample and transfer to a 400 ml. beaker. Add 25 ml. of concentrated nitric acid, place on hot plate and warm slightly. Add approximately  $\frac{1}{2}$  teaspoon potassium chlorate, place watch glasses on beakers and take to near dryness.

2. Add 10 ml. of concentrated hydrochloric acid and again place on the hot plate and take to near dryness.

3. Add 10 ml. of concentrated hydrochloric acid again and approximately 50 ml. of distilled water. Place on the hot plate, bring to a boil and boil for 5-10 minutes.

4. Remove from hot plate and filter through 15 cm. Whatman No. 40 (ashless) filter paper. Wash several times with hot distilled water.

5. Place residue in a clay annealing cup and ash in a muffle furnace.

6. Cool and weigh.

###### Calculation:

$$\frac{\text{Wt. insol in grams}}{\text{wt. sample in grams}} \times 100 = \% \text{ Acid Insol}$$

#### PREFERRED DUAL-AGENT COMBINATIONS

A.

- a. Water soluble metallic salt of a weak base of which the cation is selected from the class consisting of aluminum, cadmium, chromium, cobalt, copper, iron, calcium, magnesium, manganese, nickel and zinc, and a strong acid selected from the class consisting of hydrochloric acid, nitric acid and sulfuric acid affording the anions chloride, nitrate and sulfate, and
- b. Sodium silicate or potassium silicate.
- 5 a. Water soluble metallic salt of a weak base of which the cation is selected from the class consisting of aluminum, chromium, copper, manganese, and zinc, and a strong acid selected from the class consisting of hydrochloric acid, nitric acid and sulfuric acid affording the anions chloride, nitrate and sulfate, and
- b. Sodium hydrogen carbonate, potassium hydrogen carbonate, or ammonium hydrogen carbonate.
- C. a. Water soluble metallic salt of a weak base of which 20 the cation is selected from the class consisting of aluminum, chromium, manganese, and zinc, and a strong acid selected from the class consisting of hydrochloric acid, nitric acid and sulfuric acid affording the anions chloride, nitrate and sulfate, and
- b. Water soluble sodium monohydrogen orthophosphate, potassium monohydrogen orthophosphate, or ammonium monohydrogen orthophosphate.
- D. a. Water soluble metallic salt of a weak base of which 30 the cation is selected from the class consisting of aluminum, cobalt, copper, manganese, and zinc, and a strong acid selected from the class consisting of hydrochloric acid, nitric acid and sulfuric acid affording the anions chloride, nitrate and sulfate, and
- b. Water soluble sodium borate, potassium borate or ammonium borate.
- E. a. Water soluble metallic salt of a weak base of which 40 the cation is selected from the class consisting of aluminum, copper, and zinc, and a strong acid selected from the class consisting of hydrochloric acid, nitric acid and sulfuric acid affording the anion chloride, nitrate and sulfate, and
- b. Water soluble sodium orthophosphate, potassium orthophosphate or ammonium orthophosphate.
- F. a. Water soluble zinc chloride, zinc nitrate, or zinc sulfate, and
- b. Sodium carbonate, potassium carbonate, ammonium carbonate, sodium ferrocyanide, potassium ferrocyanide or ammonium ferrocyanide.
- G. a. Water soluble zinc chloride, zinc nitrate, or zinc sulfate, and
- b. Sodium silicate or potassium silicate.
- 55 Thus, having described the invention, what is claimed is:
1. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
- 60 1. forming a dual agent treated aqueous pulp of said ore or concentrate, said dual agent consisting essentially of
- I. (a) water soluble metallic salt of a weak base and a strong acid, and

- (b) water soluble alkali metal, water soluble alkaline earth metal or water soluble ammonium salt of a weak acid selected from the group consisting of boron acids, carbonic acids, acids of phosphorous and silicic acids; or
- II. (a) water soluble zinc salt of a strong acid, and  
(b) water soluble salt of hydroferrocyanic acid, and
2. subjecting said dual agent treated aqueous pulp to froth flotation separation whereby a molybdenite enriched concentrate is floated and hydrophobic silicate is selectively depressed into the tailings from said froth flotation separation.
2. The method of claim 1 wherein said treating of (1) is carried out by adding said metallic salt of (I) (a) and (II) (a) to said aqueous pulp prior to the addition of said salt of (I) (b) and (II) (b), as the case may be.
3. The method of claim 1 wherein said treating of (1) is carried out by adding said salt of (I) (b) and (II) (b) to said aqueous pulp prior to the addition of said metallic salt of (I) (a) and (II) (a), as the case may be.
4. The method of claim 1 wherein each component of said dual agent of (I) and (II), as the case may be, is added substantially simultaneously to said aqueous pulp.
5. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- I (a). water soluble metallic salt of a weak base of which the cation is selected from the class consisting of aluminum, cadmium, chromium, cobalt, copper, calcium, magnesium, iron, manganese, nickel and zinc, and a strong acid selected from the class consisting of hydrochloric acid, hydrofluoric acid, nitric acid and sulfuric acid affording the anions chloride, fluoride, nitrate and sulfate, and
- I (b). water soluble alkali metal, water soluble alkaline earth metal, or water soluble ammonium salt of weak acid selected from the class consisting of boron acids, carbonic acid, acids of phosphorus, and silicic acid; or
- II (a). water soluble zinc chloride, zinc fluoride, zinc nitrate, or zinc sulfate, and
- II (b). water soluble alkali metal, water soluble alkaline earth metal, or water soluble ammonium salt of hydroferrocyanic acid; and
- where said treating is carried out by adding said metallic salt of (I) (a) and (II) (a) to said aqueous pulp to condition said pulp prior to the addition of said salt of (I) (b) and (II) (b), as the case may be, and
2. subjecting said dual agent treated aqueous pulp to froth flotation separation whereby a molybdenite enriched concentrate is floated and hydrophobic silicate is selectively depressed into the tailings from said froth flotation separation.
6. The method of claim 5 wherein said aqueous pulp has a pulp density of from about 1% to 45% solids.
7. A method of separating ore or concentrate having molybdenite and a substantial amount of a hydrophobic silicate talc containing magnesium by froth flotation to obtain a molybdenite enriched concentrate and hydrophobic silicate talc enriched tailings, which method consists essentially of:
1. forming a dual agent treated aqueous pulp of said ore or concentrate,

- where the treating agent consists essentially of aluminum sulfate and sodium silicate, and
2. subjecting said dual treated aqueous pulp to froth flotation separation whereby a molybdenite enriched concentrate is floated and hydrophobic silicate talc is selectively depressed into the tailings from said froth flotation separation.
8. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- I (a). water soluble metallic salt of a weak base of which the cation is selected from the class consisting of aluminum, cadmium, chromium, cobalt, copper, calcium, magnesium, iron, manganese, nickel and zinc, and a strong acid selected from the class consisting of hydrochloric acid, hydrofluoric acid, nitric acid and sulfuric acid affording the anions chloride, fluoride, nitrate and sulfate, and
- I (b). water soluble alkali metal, water soluble alkaline earth metal, or water soluble ammonium salt of weak acid selected from the class consisting of boron acids, carbonic acid, acids of phosphorus, and silicic acid; or
- II (a). water soluble zinc chloride, zinc fluoride, zinc nitrate, or zinc sulfate, and
- II (b). water soluble alkali metal, water soluble alkaline earth metal, or water soluble ammonium salt of hydroferrocyanic acid; and
- where said treating is carried out by adding said metallic salt of (I) (a) and (II) (a) to said aqueous pulp to condition said pulp prior to the addition of said salt of (I) (b) and (II) (b), as the case may be, and
2. subjecting said dual agent treated aqueous pulp to froth flotation separation whereby a molybdenite enriched concentrate is floated and hydrophobic silicate is selectively depressed into the tailings from said froth flotation separation.
9. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- (I) (a). water soluble metallic salt of a weak base of which the cation is selected from the class consisting of aluminum, cadmium, chromium, cobalt, copper, calcium, magnesium, iron, manganese, nickel and zinc, and a strong acid selected from the class consisting of hydrochloric acid, hydrofluoric acid, nitric acid and sulfuric acid affording the anions chloride, fluoride, nitrate and sulfate, and
- (I) (b). water soluble alkali metal, water soluble alkaline earth metal, or water soluble ammonium salt of weak acid selected from the class consisting of boron acids, carbonic acid, acids of phosphorus, and silicic acid; or

## 11

- II (a). water soluble zinc chloride, zinc fluoride, zinc nitrate, or zinc sulfate, and
- II (b). water soluble alkali metal, water soluble alkaline earth metal, or water soluble ammonium salt of hydroferrocyanic acid; and
- where said aqueous pulp is treated with between about 1 and 30 pounds per ton of pulp solids of said metallic salt of (I) (a) and (II) (a) and between about 1 and 45 pounds per ton of pulp solids of said salt of (I) (b) and (II) (b) as the case may be, and
2. subjecting said dual agent treated aqueous pulp to froth flotation separation whereby a molybdenite enriched concentrate is floated and hydrophobic silicate is selectively depressed into the tailings from said froth flotation separation.
- 10 15 20 25 30 35 40 45 50 55 60 65
10. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- a. water soluble metallic salt of a weak base of which the cation is selected from the class consisting of aluminum, cadmium, chromium, cobalt, copper, calcium, magnesium, iron, manganese, nickel and zinc, and a strong acid selected from the class consisting of hydrochloric acid, nitric acid and sulfuric acid affording the anions chloride, nitrate and sulfate, and
  - b. sodium silicate or potassium silicate and
2. subjecting said dual agent treated aqueous pulp to froth flotation separation whereby a molybdenite enriched concentrate is floated and hydrophobic silicate is selectively depressed into the tailings from said froth flotation separation.
11. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- a. water soluble metallic salt of a weak base of which the cation is selected from the class consisting of aluminum, chromium, copper, manganese, and zinc, and a strong acid selected from the class consisting of hydrochloric acid, nitric acid and sulfuric acid affording the anions chloride, nitrate and sulfate, and
  - b. sodium hydrogen carbonate, potassium hydrogen carbonate, or ammonium hydrogen carbonate, and
2. subjecting said dual agent treated aqueous pulp to froth flotation separation whereby a molybdenite enriched concentrate is floated and hydrophobic silicate is selectively depressed into the tailings from said froth flotation separation.
12. A method of separating ore or concentrate having molybdenite and a substantial amount of hydrophobic silicate containing magnesium by froth flotation to obtain a molybdenite enriched concentrate and hydro-

## 12

- phobic silicate enriched tailings, which method consists essentially of:
1. forming a dual agent treated aqueous pulp of said ore or concentrate,
- where the treating agent consists essentially of
- a. water soluble metallic salt of a weak base of which the cation is selected from the class consisting of aluminum, chromium, manganese, and zinc, and a strong acid selected from the class consisting of hydrochloric acid, nitric acid and sulfuric acid affording the anions chloride, nitrate and sulfate, and
  - b. water soluble sodium monohydrogen orthophosphate, potassium monohydrogen orthophosphate, or ammonium monohydrogen orthophosphate, and
2. subjecting said dual agent treated aqueous pulp to froth flotation separation whereby a molybdenite enriched concentrate is floated and hydrophobic silicate is selectively depressed into the tailings from said froth flotation separation.
13. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- a. water soluble metallic salt of a weak base of which the cation is selected from the class consisting of aluminum, cobalt, copper, manganese, and zinc, and a strong acid selected from the class consisting of hydrochloric acid, nitric acid and sulfuric acid affording the anions chloride, nitrate and sulfate, and
  - b. water soluble sodium borate, potassium borate or ammonium borate, and
2. subjecting said dual agent treated aqueous pulp to froth flotation separation whereby a molybdenite enriched concentrate is floated and hydrophobic silicate is selectively depressed into the tailings from said froth flotation separation.
14. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:
1. forming a dual agent treated aqueous pulp of said ore or concentrate,
- where the treating agent consists essentially of
- a. water soluble metallic salt of a weak base of which the cation is selected from the class consisting of aluminum, copper, and zinc, and a strong acid selected from the class consisting of hydrochloric acid, nitric acid and sulfuric acid affording the anions chloride, nitrate and sulfate, and
  - b. water soluble sodium orthophosphate, potassium orthophosphate, or ammonium orthophosphate, and
2. subjecting said dual agent treated aqueous pulp to froth flotation separation whereby a molybdenite enriched concentrate is floated and hydrophobic silicate is selectively depressed into the tailings from said froth flotation separation.

15. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:

1. forming a dual agent treated aqueous pulp of said ore or concentrate,

where the treating agent consists essentially of

- a. water soluble zinc chloride, zinc nitrate or zinc sulfate, and
- b. sodium carbonate, potassium carbonate, ammonium carbonate, sodium ferrocyanide, potassium ferrocyanide or ammonium ferrocyanide, and

2. subjecting said dual agent treated aqueous pulp to froth flotation separation whereby a molybdenite enriched concentrate is floated and hydrophobic silicate is selectively depressed into the tailings from said froth flotation separation.

16. A method of separating ore or concentrate having molybdenite and a substantial amount of hydrophobic silicate containing magnesium by froth flotation to obtain a molybdenite enriched concentrate and hydrophobic silicate enriched tailings, which method consists essentially of:

1. forming a dual agent treated aqueous pulp of said ore or concentrate,

where the treating agent consists essentially of

- a. water soluble zinc chloride, zinc nitrate, or zinc sulfate, and
- b. sodium silicate or potassium silicate, and

2. subjecting said dual agent treated aqueous pulp to froth flotation separation whereby a molybdenite enriched concentrate is floated and hydrophobic silicate is selectively depressed into the tailings from said froth flotation separation.

17. A method of separating a charge of molybdenite concentrate containing molybdenite as the major metal value, talc and other acid insoluble minerals which method consists essentially of:

1. forming an aqueous pulp to said concentrate;
2. adding zinc sulfate to said aqueous pulp and mixing for a conditioning time followed by the addition of sodium silicate, and
3. subjecting said admixture to froth flotation separation whereby a molybdenite enriched concentrate product is floated and talc is selectively depressed

into the tailings from said froth flotation separation.

18. The method of claim 17 wherein said charge concentrate contains about 18% molybdenite, 4% chalcopyrite, 5% pyrite and 69% acid insoluble minerals of which a major portion is a hydrophobic talc,

sodium silicate is added in an amount of about 7.5 pounds per ton of solids and zinc sulfate is added in an amount of about 16 pounds per ton of solids; and the conditioning time is about 30 minutes.

19. A method of separating molybdenite concentrate containing molybdenite as the major metal value, talc and other acid insoluble minerals, which method consists essentially of:

1. forming an aqueous pulp of said concentrate;
2. conditioning said aqueous pulp with aluminum sulfate;
3. adding to said conditioned pulp sodium acid carbonate; and
4. subjecting said conditioned aqueous pulp to froth flotation separation whereby a molybdenite enriched concentrate is floated and talc is selectively depressed into the tailings from said froth flotation separation.

20. The method of claim 19 wherein said aluminum sulfate is added in an amount of about 1 pound per ton of solids and said carbonate is added in an amount of about 7.5 pounds per ton of solids.

21. A method of separating molybdenite concentrate containing molybdenite as the major metal value, talc and other acid insoluble minerals, which method consists essentially of:

1. forming an aqueous pulp of said concentrate;
2. conditioning said aqueous pulp with zinc sulfate;
3. adding to said conditioned pulp potassium ferrocyanide; and
4. subjecting said sulfate-ferrocyanide treated pulp to froth flotation separation whereby a molybdenite enriched concentrate is floated and talc is selectively depressed into the tailings from said froth flotation separation.

22. The method of claim 21 wherein said zinc sulfate is added in an amount of about 6 pounds per ton of solids and said ferrocyanide is added in an amount of about 8 pounds per ton of solids.

\* \* \* \* \*